

## UNITED STATES PATENT OFFICE

2,346,065

PRODUCTION OF NEUTRAL TONES IN  
PHOTOGRAPHIC EMULSIONSBurt H. Carroll and Cyril J. Staud, Rochester,  
N. Y., assignors to Eastman Kodak Company,  
Rochester, N. Y., a corporation of New JerseyNo Drawing. Application September 23, 1941,  
Serial No. 411,976

8 Claims. (Cl. 95—6)

This invention relates to photographic emulsions and particularly to a method for the formation of neutral tones in such emulsions.

It is known that the developed image of fine grain emulsions is rarely neutral in color, being generally a brownish or warm tone. For many materials this is considered objectionable and the use of compounds in the developer or the emulsion to produce a neutral tone is old. Many materials, including thiohydantoin and alkylated thiohydantoins have been suggested for this purpose. These materials, however, are not always effective to produce neutral tones in emulsions.

It is, therefore, the principal object of the present invention to provide a novel method for the production of neutral tones in photographic emulsions. A further object is to provide a method for the production of neutral tones in fine grain emulsions. A still further object is to provide novel compounds for producing neutral tones in bromide or bromoiodide emulsions.

These objects are accomplished by incorporating in the emulsion or in a photographic developer an aryl substituted thiohydantoin. These compounds are especially effective in the case of bromide or bromoiodide emulsions whereas many of the previously used compounds are effective only with chloride emulsions.

The aryl substituted thiohydantoins used according to our invention may be added to the developer or introduced into the emulsion before the development. The introduction of the material into the emulsion may be carried out by adding it to the emulsion at any stage after the ripening process. Since the compounds are capable of reacting with silver salts to form silver sulfide, they should not be added to the emulsion before or during the ripening process. They may be added to the emulsion at any subsequent stage in its manufacture such as by mixing a solution of the agent with the emulsion before coating.

The amount of arylated thiohydantoin to be added to the emulsion may vary considerably depending upon the composition of the compound and of the emulsion and the degree to which the tone is to be changed. The compounds are preferably added to the finished emulsions in small amounts of the order of 30 milligrams per liter of emulsion containing 40 grams of silver bromide per liter.

Compounds suitable for use according to our invention include arylated thiohydantoins such as 1,3-diphenyl-2-thiohydantoin.



Our invention may be illustrated by the following example:

20 A gelatin silver bromide emulsion was prepared in a normal manner, as described in the literature, a non-ammonia type being used. The emulsion in which the example was obtained was a fine-grain, moderate contrast material of low speed. The 1,3-diphenyl-2-thiohydantoin was effective in emulsions of the type described above, containing somewhat higher iodide content than is frequently used in the preparation of fine grain materials.

30 It will be understood that the examples included herein are illustrative only and that other compounds falling within the scope of the appended claims may be used in our process.

We claim:

1. The method for producing neutral tones in gelatino-silver halide emulsions which comprises ripening the emulsion and adding to it thereafter an aryl substituted thiohydantoin.
2. The method for producing neutral tones in gelatino-silver bromide emulsions which comprises ripening the emulsion and adding to it thereafter an aryl substituted thiohydantoin.
3. The method for producing neutral tones in gelatino-silver bromide emulsions which comprises ripening the emulsion and adding to it a diaryl substituted 2-thiohydantoin.
4. The method for producing neutral tones in gelatino silver bromide emulsions which comprises ripening the emulsion and adding to it a 50 N-diphenyl-2-thiohydantoin.

5. The method for producing neutral tones in gelatino-silver halide emulsions which comprises ripening the emulsion and adding to it 1,3-diphenyl-2-thiohydantoin.

6. The method for producing neutral tones in gelatino silver bromide emulsions which comprises ripening the emulsion and adding to it 1,3-diphenyl-2-thiohydantoin.

7. A ripened silver halide photographic emul-

sion capable of producing neutral tones on development, containing a N-diphenyl-2-thiohydantoin added after ripening.

8. A ripened silver halide photographic emulsion capable of producing neutral tones on development containing 1,3-diphenyl - 2 - thiohydantoin added after ripening.

BURT H. CARROLL.  
CYRIL J. STAUD.